

## UNITED STATES PATENT OFFICE

2,005,113

## PRODUCT FOR TREATING BITUMENS

Orvall Smiley, Indianapolis, Ind.

No Drawing. Application March 30, 1933,  
Serial No. 663,651

## 1 Claim. (Cl. 134—1)

This invention relates to a composition which may be prepared by skilled operators at a central point to be shipped out to local points to be mixed with bitumens for the purpose of producing metamorphic change in the bitumens to increase their ductility and tenacity or adhesiveness.

A primary object of my invention is to provide a product for the above indicated purpose which may be used by unskilled labor to produce the metamorphosed bitumen as the end product, all without technical or closely supervised steps, but at the same time will give a constant, uniform and stable end product. A further important object is to provide a product of the nature indicated which may have small volume so that the cost of shipment may be small when the end product is to be utilized in its metamorphosed condition.

It is known that bitumens are continuously but slowly undergoing metamorphic changes throughout time, but it is my purpose to bring about metamorphic changes quickly and under control.

When the metamorphic compound forming my invention is used, through metamorphosis of the bitumen, various usable bitumens of varying qualities are produced.

To produce this metamorphic agent or compound, to fifteen parts of a fatty acid such as oleic, stearic acid or the like, and fifteen parts of soap of sodium, potassium, or ammonium base, I add one hundred twenty parts of a mutual solvent therefor, preferably "Tetralin" which is beta-tetra-hydro-naphthalene, all while heated. Other solvents may be employed, such as monoethyl ether or ethylene glycol, the monobutyl ether of ethylene glycol, monoethyl ether of diethylene glycol, ethyl and isopropyl alcohols, and the like.

The metamorphic agent thus formed may be stored and shipped for use at any given place or plant. To use it, it is simply poured into the bitumen, the mixture being heated and preferably agitated. As is well known, a considerable variation is found in bitumens as to their charac-

teristics. The proportions of metamorphic compound and bitumen will depend upon the particular bitumen employed. Knowing the specifications of the particular bitumen selected, then the amount of the metamorphic compound to be used to obtain a desired metamorphosed bitumen is determined. For example, take the bitumen known to the trade as "Texaco" No. 115, this bitumen at 77 degrees F. has a specific gravity of 1.00; penetration in 5 seconds by 100 gram weight of not less than 100 millimeters nor more than 120; flash point not less than 420 degrees F.; fire point not less than 520 degrees F.; solubility of 99.5% in carbon disulphide and 99.5% in carbon tetrachloride; and ductility (Dow method) not less than 50 centimeters.

Take 996 grams of this bitumen, and add thereto 170 grams of the metamorphic compound as above indicated. Heat the mixture to below the boiling points of the ingredients and agitate. The end product thus formed is ready for use. The end product is substantially stable. By varying the amount of the metamorphic compound in proportion to the bitumen used varying degrees of metamorphosis are produced.

The solvent "Tetralin" and other like substances serve as a metamorphic agent between the fatty acid and the soap to create the new metamorphic agent which constitutes my invention and it is this new agent which then is the metamorphic agent for metamorphosing the bitumen.

I claim:

A preparative unmulsified product to be added to bitumens to set up a change therein to render the bitumens suitable for roadways, said product consisting of substantially 15 parts higher aliphatic fatty acids, 15 parts soap, and 120 parts of beta tetrahydronaphthalene, and forming a stable product giving uniform results regardless of storage periods when applied to said bitumens, said tetrahydronaphthalene, in the presence of said acid and soap, operating to cause said change.

ORVALL SMILEY.